



US009315753B2

(12) **United States Patent**  
**Reid**

(10) **Patent No.:** **US 9,315,753 B2**  
(45) **Date of Patent:** **\*Apr. 19, 2016**

(54) **DIESEL FUEL COMPOSITIONS**

(75) Inventor: **Jacqueline Reid**, Cymau (GB)

(73) Assignee: **Innospec Limited** (GB)

(\*) Notice: Subject to any disclaimer, the term of this patent is extended or adjusted under 35 U.S.C. 154(b) by 0 days.

This patent is subject to a terminal disclaimer.

(21) Appl. No.: **14/236,764**

(22) PCT Filed: **Aug. 2, 2012**

(86) PCT No.: **PCT/GB2012/051879**

§ 371 (c)(1),

(2), (4) Date: **Feb. 24, 2014**

(87) PCT Pub. No.: **WO2013/017887**

PCT Pub. Date: **Feb. 7, 2013**

(65) **Prior Publication Data**

US 2014/0174391 A1 Jun. 26, 2014

(30) **Foreign Application Priority Data**

Aug. 3, 2011 (EP) ..... 11176494

(51) **Int. Cl.**

**C10L 1/22** (2006.01)  
**C10L 10/04** (2006.01)

(Continued)

(52) **U.S. Cl.**

CPC ..... **C10L 10/04** (2013.01); **C10L 1/221** (2013.01); **C10L 1/2225** (2013.01); **C10L 1/234** (2013.01); **C10L 1/238** (2013.01); **C10L 1/2383** (2013.01); **C10L 1/2387** (2013.01); **C10L 10/06** (2013.01); **C10L 1/22** (2013.01); **C10L 1/226** (2013.01); **C10L 10/18** (2013.01);

(Continued)

(58) **Field of Classification Search**

CPC ... C10L 1/221; C10L 1/222; C10L 2230/08;  
C10L 2230/22

USPC ..... 44/422, 415  
See application file for complete search history.

(56) **References Cited**

U.S. PATENT DOCUMENTS

3,018,250 A 1/1962 Anderson et al.  
3,172,892 A 3/1965 Le Suer et al.

(Continued)

FOREIGN PATENT DOCUMENTS

EP 0565285 A1 10/1993  
EP 0831141 A1 3/1998

(Continued)

OTHER PUBLICATIONS

International Preliminary Report on Patentability for International Application No. PCT/GB2012/051879 dated Feb. 4, 2014.

*Primary Examiner* — Ellen McAvoy

(74) *Attorney, Agent, or Firm* — Burns & Levinson LLP;  
Janine M. Susan

(57) **ABSTRACT**

A diesel fuel composition comprising, as an additive, the product of a Mannich reaction between: (a) an aldehyde; (b) an amine; and (c) a substituted phenol; wherein the phenol is substituted with at least one branched hydrocarbyl group having a molecular weight of between 200 and 3000; and wherein in the Mannich reaction used to form the additive the molar ratio of component (a) to component (b) is 2.2-1.01:1; the molar ratio of component (a) to component (c) is 1.99-1.01:1 and the molar ratio of component (b) to component (c) is 1:1.01-1.99.

**11 Claims, 7 Drawing Sheets**

→ 75ppm additive A



|      |                    |                                                                                                                                   |                   |         |                        |         |
|------|--------------------|-----------------------------------------------------------------------------------------------------------------------------------|-------------------|---------|------------------------|---------|
| (51) | <b>Int. Cl.</b>    |                                                                                                                                   | 5,876,468 A *     | 3/1999  | Moreton .....          | 44/415  |
|      | <i>C10L 1/222</i>  | (2006.01)                                                                                                                         | 6,117,198 A *     | 9/2000  | Moreton .....          | 44/415  |
|      | <i>C10L 1/234</i>  | (2006.01)                                                                                                                         | 7,112,230 B2 *    | 9/2006  | Malfer et al. .....    | 44/415  |
|      | <i>C10L 1/238</i>  | (2006.01)                                                                                                                         | 7,597,726 B2 *    | 10/2009 | Hou et al. .....       | 44/415  |
|      | <i>C10L 1/2383</i> | (2006.01)                                                                                                                         | 7,906,470 B2 *    | 3/2011  | Stevenson et al. ..... | 508/542 |
|      | <i>C10L 1/2387</i> | (2006.01)                                                                                                                         | 7,947,093 B2 *    | 5/2011  | Barton et al. .....    | 44/422  |
|      | <i>C10L 10/06</i>  | (2006.01)                                                                                                                         | 7,951,211 B2 *    | 5/2011  | Barton et al. .....    | 44/422  |
|      | <i>C10L 1/226</i>  | (2006.01)                                                                                                                         | 8,147,569 B2 *    | 4/2012  | Barton et al. .....    | 44/422  |
|      | <i>C10L 10/18</i>  | (2006.01)                                                                                                                         | 8,557,003 B2 *    | 10/2013 | Malfer et al. .....    | 44/415  |
|      |                    |                                                                                                                                   | 8,715,375 B2 *    | 5/2014  | Reid .....             | 44/415  |
| (52) | <b>U.S. Cl.</b>    |                                                                                                                                   | 2003/0172582 A1   | 9/2003  | Carabell et al.        |         |
|      | CPC                | <i>C10L 2200/0446</i> (2013.01); <i>C10L 2200/0476</i> (2013.01); <i>C10L 2200/0492</i> (2013.01); <i>C10L 2270/026</i> (2013.01) | 2008/0141583 A1 * | 6/2008  | Malfer et al. .....    | 44/415  |

## FOREIGN PATENT DOCUMENTS

|    |               |        |
|----|---------------|--------|
| EP | 1344785 A1    | 9/2003 |
| WO | 0009634 A1    | 2/2000 |
| WO | 2007015080 A1 | 2/2007 |
| WO | 2009040583 A1 | 4/2009 |
| WO | 2009040584 A1 | 4/2009 |
| WO | 2010097624 A1 | 9/2010 |

\* cited by examiner

(56) **References Cited**

## U.S. PATENT DOCUMENTS

3,231,587 A 1/1966 Rense  
 3,361,673 A 1/1968 Stuart et al.



FIGURE 1



FIGURE 2



FIGURE 3



FIGURE 4



FIGURE 5



FIGURE 6



FIGURE 7

## 1

## DIESEL FUEL COMPOSITIONS

## CROSS-REFERENCE TO RELATED APPLICATIONS

This application is a U.S. national stage application under 35 U.S.C. 371 of co-pending International Application No. PCT/GB2012/051879 filed on Aug. 2, 2012 and entitled FUEL COMPOSITIONS, which in turn claims priority to European Patent Application No. 11176494.0, filed on Aug. 3, 2011, which is incorporated by reference herein in its entirety for all purposes.

## BRIEF DESCRIPTION OF THE DRAWINGS

FIG. 1 is a graph of observed change in engine power over time using fuel containing Additive A of the invention.

FIG. 2 is a graph of observed change in engine power over time using fuel containing comparative Additive B not of the invention.

FIG. 3 is a graph of observed change in engine power over time using fuel containing comparative Additive C not of the invention.

FIG. 4 is a graph of observed change in engine power over time using fuel containing comparative Additive D not of the invention.

FIG. 5 is a graph of observed change in engine power over time using fuel containing comparative Additive E not of the invention.

FIG. 6 is a graph of observed change in engine power over time using fuel containing comparative Additive F not of the invention.

FIG. 7 is a graph of clean-up performance showing restoration of engine power using fuel containing Additive G of the invention.

The present invention relates to fuel compositions and additives thereto. In particular the invention relates to additives for diesel fuel compositions, especially those suitable for use in modern diesel engines with high pressure fuel systems.

Due to consumer demand and legislation, diesel engines have in recent years become much more energy efficient, show improved performance and have reduced emissions.

These improvements in performance and emissions have been brought about by improvements in the combustion process. To achieve the fuel atomisation necessary for this improved combustion, fuel injection equipment has been developed which uses higher injection pressures and reduced fuel injector nozzle hole diameters. The fuel pressure at the injection nozzle is now commonly in excess of 1500 bar ( $1.5 \times 10^8$  Pa). To achieve these pressures the work that must be done on the fuel also increases the temperature of the fuel. These high pressures and temperatures can cause degradation of the fuel.

Diesel engines having high pressure fuel systems can include but are not limited to heavy duty diesel engines and smaller passenger car type diesel engines. Heavy duty diesel engines can include very powerful engines such as the MTU series 4000 diesel having 20 cylinder variants designed primarily for ships and power generation with power output up to 4300 kW or engines such as the Renault dXi 7 having 6 cylinders and a power output around 240 kW. A typical passenger car diesel engine is the Peugeot DW10 having 4 cylinders and power output of 100 kW or less depending on the variant.

In all of the diesel engines relating to this invention, a common feature is a high pressure fuel system. Typically

## 2

pressures in excess of 1350 bar ( $1.35 \times 10^8$  Pa) are used but often pressures of up to 2000 bar ( $2 \times 10^8$  Pa) or more may exist.

Two non-limiting examples of such high pressure fuel systems are: the common rail injection system, in which the fuel is compressed utilizing a high-pressure pump that supplies it to the fuel injection valves through a common rail; and the unit injection system which integrates the high-pressure pump and fuel injection valve in one assembly, achieving the highest possible injection pressures exceeding 2000 bar ( $2 \times 10^8$  Pa). In both systems, in pressurising the fuel, the fuel gets hot, often to temperatures around 100° C., or above.

In common rail systems, the fuel is stored at high pressure in the central accumulator rail or separate accumulators prior to being delivered to the injectors. Often, some of the heated fuel is returned to the low pressure side of the fuel system or returned to the fuel tank. In unit injection systems the fuel is compressed within the injector in order to generate the high injection pressures. This in turn increases the temperature of the fuel.

In both systems, fuel is present in the injector body prior to injection where it is heated further due to heat from the combustion chamber. The temperature of the fuel at the tip of the injector can be as high as 250-350° C.

Thus the fuel is stressed at pressures from 1350 bar ( $1.35 \times 10^8$  Pa) to over 2000 bar ( $2 \times 10^8$  Pa) and temperatures from around 100° C. to 350° C. prior to injection, sometimes being recirculated back within the fuel system thus increasing the time for which the fuel experiences these conditions.

A common problem with diesel engines is fouling of the injector, particularly the injector body, and the injector nozzle. Fouling may also occur in the fuel filter. Injector nozzle fouling occurs when the nozzle becomes blocked with deposits from the diesel fuel. Fouling of fuel filters may be related to the recirculation of fuel back to the fuel tank. Deposits increase with degradation of the fuel. Deposits may take the form of carbonaceous coke-like residues or sticky or gum-like residues. Diesel fuels become more and more unstable the more they are heated, particularly if heated under pressure. Thus diesel engines having high pressure fuel systems may cause increased fuel degradation.

The problem of injector fouling may occur when using any type of diesel fuels. However, some fuels may be particularly prone to cause fouling or fouling may occur more quickly when these fuels are used. For example, fuels containing biodiesel have been found to produce injector fouling more readily. Diesel fuels containing metallic species may also lead to increased deposits. Metallic species may be deliberately added to a fuel in additive compositions or may be present as contaminant species. Contamination occurs if metallic species from fuel distribution systems, vehicle distribution systems, vehicle fuel systems, other metallic components and lubricating oils become dissolved or dispersed in fuel.

Transition metals in particular cause increased deposits, especially copper and zinc species. These may be typically present at levels from a few ppb (parts per billion) up to 50 ppm, but it is believed that levels likely to cause problems are from 0.1 to 50 ppm, for example 0.1 to 10 ppm.

When injectors become blocked or partially blocked, the delivery of fuel is less efficient and there is poor mixing of the fuel with the air. Over time this leads to a loss in power of the engine, increased exhaust emissions and poor fuel economy.

As the size of the injector nozzle hole is reduced, the relative impact of deposit build up becomes more significant.

By simple arithmetic a 5 µm layer of deposit within a 500 µm hole reduces the flow area by 4% whereas the same 5 µm layer of deposit in a 200 µm hole reduces the flow area by 9.8%.

At present, nitrogen-containing detergents may be added to diesel fuel to reduce coking. Typical nitrogen-containing detergents are those formed by the reaction of a polyisobutylene-substituted succinic acid derivative with a polyalkylene polyamine. However, newer engines including finer injector nozzles are more sensitive and current diesel fuels may not be suitable for use with the new engines incorporating these smaller nozzle holes.

The present inventor has developed diesel fuel compositions which when used in diesel engines having high pressure fuel systems provide improved performance compared with diesel fuel compositions of the prior art.

It is advantageous to provide a diesel fuel composition which prevents or reduces the occurrence of deposits in a diesel engine. Such fuel compositions may be considered to perform a "keep clean" function i.e. they prevent or inhibit fouling.

However it would also be desirable to provide a diesel fuel composition which would help clean up deposits that have already formed in an engine, in particular deposits which have formed on the injectors. Such a fuel composition which when combusted in a diesel engine removes deposits therefrom thus effecting the "clean-up" of an already fouled engine.

As with "keep clean" properties, "clean-up" of a fouled engine may provide significant advantages. For example, superior clean up may lead to an increase in power and/or an increase in fuel economy. In addition removal of deposits from an engine, in particular from injectors may lead to an increase in interval time before injector maintenance or replacement is necessary thus reducing maintenance costs.

Although for the reasons mentioned above deposits on injectors is a particular problem found in modern diesel engines with high pressure fuel systems, it is desirable to provide a diesel fuel composition which also provides effective detergency in older traditional diesel engines such that a single fuel supplied at the pumps can be used in engines of all types.

It is also desirable that fuel compositions reduce the fouling of vehicle fuel filters. It would be useful to provide compositions that prevent or inhibit the occurrence of fuel filter deposits i.e. provide a "keep clean" function. It would be useful to provide compositions that remove existing deposits from fuel filter deposits i.e. provide a "clean up" function. Compositions able to provide both of these functions would be especially useful.

The applicant has previously found that additives formed by the Mannich reaction of an aldehyde, an amine and a low molecular weight phenol, for example dodecyl phenol, can be useful in reducing deposits in modern diesel engines. Such additives are described in WO 2010/097624 and WO 2009/040584. However when the applicant prepared additives by the Mannich reaction of an aldehyde, an amine and a phenol having a branched hydrocarbyl substituent using the same reactant ratios as previously used the performance of the additives was found to be inferior.

According to a first aspect of the present invention there is provided a diesel fuel composition comprising, as an additive, the product of a Mannich reaction between:

- (a) an aldehyde;
- (b) an amine; and
- (c) a substituted phenol;

wherein the phenol is substituted with at least one branched hydrocarbyl group having a molecular weight of between 200 and 3000; and wherein in the Mannich reaction used to form the additive the molar ratio of component (a) to component

(b) is 2.2-1.01:1; the molar ratio of component (a) to component (c) is 1.99-1.01:1 and the molar ratio of component (b) to component (c) is 1:1.01-1.99.

Any aldehyde may be used as aldehyde component (a) of the Mannich additive. Preferably the aldehyde component (a) is an aliphatic aldehyde. Preferably the aldehyde has 1 to 10 carbon atoms, preferably 1 to 6 carbon atoms, more preferably 1 to 3 carbon atoms. Most preferably the aldehyde is formaldehyde.

10 Amine component (b) of the Mannich additive may be at least one amino or polyamino compound having at least one NH group. Suitable amino compounds include primary or secondary monoamines having hydrocarbon substituents of 1 to 30 carbon atoms or hydroxyl-substituted hydrocarbon substituents of 1 to about 30 carbon atoms.

In preferred embodiments the amine component (b) is a polyamine.

Polyamines may be selected from any compound including 20 two or more amine groups. Preferably the polyamine is a (poly)alkylene polyamine (by which is meant an alkylene polyamine or a polyalkylene polyamine; including in each case a diamine, within the meaning of "polyamine"). Preferably the polyamine is a (poly)alkylene polyamine in which 25 the alkylene component has 1 to 6, preferably 1 to 4, most preferably 2 to 3 carbon atoms. Most preferably the polyamine is a (poly)ethylene polyamine (that is, an ethylene polyamine or a polyethylene polyamine).

Preferably the polyamine has 2 to 15 nitrogen atoms, preferably 2 to 10 nitrogen atoms, more preferably 2 to 8 nitrogen atoms.

Preferably the polyamine component (b) includes the moiety  $R^1R^2NCHR^3CHR^4NR^5R^6$  wherein each of  $R^1$ ,  $R^2$ ,  $R^3$ ,  $R^4$ ,  $R^5$  and  $R^6$  is independently selected from hydrogen, and an optionally substituted alkyl, alkenyl, alkynyl, aryl, alkylaryl or arylalkyl substituent.

Thus the polyamine reactants used to make the Mannich reaction products of the present invention preferably include 40 an optionally substituted ethylene diamine residue.

Preferably at least one of  $R^1$  and  $R^2$  is hydrogen. Preferably both of  $R^1$  and  $R^2$  are hydrogen.

Preferably at least two of  $R^1$ ,  $R^2$ ,  $R^5$  and  $R^6$  are hydrogen.

Preferably at least one of  $R^3$  and  $R^4$  is hydrogen. In some 45 preferred embodiments each of  $R^3$  and  $R^4$  is hydrogen. In some embodiments  $R^3$  is hydrogen and  $R^4$  is alkyl, for example  $C_1$  to  $C_4$  alkyl, especially methyl.

Preferably at least one of  $R^5$  and  $R^6$  is an optionally substituted alkyl, alkenyl, alkynyl, aryl, alkylaryl or arylalkyl 50 substituent.

In embodiments in which at least one of  $R^1$ ,  $R^2$ ,  $R^3$ ,  $R^4$ ,  $R^5$  and  $R^6$  is not hydrogen, each is independently selected from an optionally substituted alkyl, alkenyl, alkynyl, aryl, alkylaryl or arylalkyl moiety. Preferably each is independently 55 selected from hydrogen and an optionally substituted C(1-6) alkyl moiety.

In particularly preferred compounds each of  $R^1$ ,  $R^2$ ,  $R^3$ ,  $R^4$  and  $R^5$  is hydrogen and  $R^6$  is an optionally substituted alkyl, alkenyl, alkynyl, aryl, alkylaryl or arylalkyl substituent. Preferably  $R^6$  is an optionally substituted C(1-6) alkyl moiety.

Such an alkyl moiety may be substituted with one or more groups selected from hydroxyl, amino (especially unsubstituted amino;  $—NH—$ ,  $—NH_2$ ), sulpho, sulphony, C(1-4) alkoxy, nitro, halo (especially chloro or fluoro) and mercapto.

60 There may be one or more heteroatoms incorporated into the alkyl chain, for example O, N or S, to provide an ether, amine or thioether.

Especially preferred substituents R<sup>1</sup>, R<sup>2</sup>, R<sup>3</sup>, R<sup>4</sup>, R<sup>5</sup> or R<sup>6</sup> are hydroxy-C(1-4)alkyl and amino-(C(1-4)alkyl, especially HO—CH<sub>2</sub>—CH<sub>2</sub>— and H<sub>2</sub>N—CH<sub>2</sub>—CH<sub>2</sub>—.

Suitably the polyamine includes only amine functionality, or amine and alcohol functionalities.

The polyamine may, for example, be selected from ethylenediamine, diethylenetriamine, triethylenetetramine, tetraethylenepentamine, pentaethylenhexamine, hexaethylenepentamine, heptaethylenoctamine, propane-1,2-diamine, 2(2-amino-ethylamino)ethanol, and N',N'-bis(2-aminoethyl)ethylenediamine (N(CH<sub>2</sub>CH<sub>2</sub>NH<sub>2</sub>)<sub>3</sub>). Most preferably the polyamine comprises tetraethylenepentamine or ethylenediamine.

Commercially available sources of polyamines typically contain mixtures of isomers and/or oligomers, and products prepared from these commercially available mixtures fall within the scope of the present invention.

The polyamines used to form the Mannich additives of the present invention may be straight chained or branched, and may include cyclic structures.

Phenol component (c) used to prepare the Mannich additives of the present invention may be substituted with 1 to 4 groups on the aromatic ring (in addition to the phenol OH). For example it may be a tri- or di-substituted phenol. Most preferably component (c) is a mono-substituted phenol. Substitution may be at the ortho, and/or meta, and/or para position(s).

Each phenol moiety may be ortho, meta or para substituted with the aldehyde/amine residue. Compounds in which the aldehyde residue is ortho or para substituted are most commonly formed. Mixtures of compounds may result. In preferred embodiments the starting phenol is para substituted and thus the ortho substituted product results.

The phenol may be substituted with any common group, for example one or more of an alkyl group, an alkenyl group, an alkynyl group, a nitryl group, a carboxylic acid, an ester, an ether, an alkoxy group, a halo group, a further hydroxyl group, a mercapto group, an alkyl mercapto group, an alkyl sulphoxy group, a sulphonyl group, an aryl group, an arylalkyl group, a substituted or unsubstituted amine group or a nitro group.

As mentioned above the phenol includes at least one branched hydrocarbyl substituent. The hydrocarbyl substituent may be optionally substituted with, for example, hydroxyl, halo, (especially chloro and fluoro), alkoxy, alkyl, mercapto, alkyl sulphoxy, aryl or amino residues. Preferably the hydrocarbyl group consists essentially of carbon and hydrogen atoms. The substituted phenol may include an alkenyl or alkynyl residue including one or more double and/or triple bonds.

The hydrocarbyl-based substituents are preferably predominantly saturated, that is, they contain no more than one carbon-to-carbon unsaturated bond for every ten carbon-to-carbon single bonds present. Most preferably they contain no more than one carbon-to-carbon unsaturated bond for every 50 carbon-to-carbon bonds present.

Preferably component (c) is a monoalkyl phenol, especially a para-substituted monoalkyl phenol in which the alkyl chain of the substituent is branched.

In preferred embodiments phenol component (c) used to prepare Mannich reaction product additive (ii) includes a predominantly or completely saturated branched hydrocarbyl substituent. Preferably this predominantly or completely saturated hydrocarbyl substituent is branched along the length of the chain. By branched along the length of the chain we mean that there are multiple branches from the main (or longest) chain. Preferably there is a branch at least every 10

carbon atoms along the main chain, preferably at least every 6 carbons, suitably at least every 4 carbons, for example every 3 carbon atoms or every 2 carbon atoms.

A particular carbon atom in the main hydrocarbyl chain (which is preferably an alkylene chain) may have one or two branching hydrocarbyl groups. By branching hydrocarbyl groups we mean hydrocarbyl groups not forming part of the main chain but directly attached thereto. Thus the main hydrocarbyl chain may include the moiety —CHR<sup>1</sup>— or —CR<sup>1</sup>R<sup>2</sup>— wherein R<sup>1</sup> and R<sup>2</sup> are branching hydrocarbyl groups.

Preferably each branching hydrocarbyl group is an alkyl group, preferably a C<sub>1</sub> to C<sub>4</sub> alkyl group, for example propyl, ethyl or most preferably methyl.

In some preferred embodiments phenol component (c) used to prepare Mannich reaction product additive (ii) includes a hydrocarbyl substituent which is substituted with methyl groups along the main chain thereof. Suitably there are a plurality of carbon atoms which each have two methyl substituents.

Preferably the branching points are substantially equally spaced along the main chain of the hydrocarbyl group of phenol component (c).

Component (c) used to prepare additive (ii) includes at least one branched hydrocarbyl substituent. Preferably this is an alkyl substituent. In especially preferred embodiments the hydrocarbyl substituent is derived from a polyalkene, suitably a polymer of a branched alkene, for example polyisobutene or polypropene.

In especially preferred embodiments component (c) used in the preparation of Mannich reaction product additive (ii) includes a poly(isobutene) derived substituent.

Thus the Mannich reaction product additives used in the present invention preferably include a hydrocarbyl chain having the repeating unit:



Poly(isobutenes) are prepared by the addition polymerisation of isobutene, (CH<sub>3</sub>)<sub>2</sub>C=CH<sub>2</sub>. Each molecule of the resulting polymer will include a single alkene moiety.

Conventional polyisobutenes and so-called "highly-reactive" polyisobutenes are suitable for use in preparing additive (i) of the present invention. Highly reactive polyisobutenes in this context are defined as polyisobutenes wherein at least 50%, preferably 70% or more, of the terminal olefinic double bonds are of the vinylidene type as described in EP0565285. Particularly preferred polyisobutenes are those having more than 80 mol % and up to 100% of terminal vinylidene groups such as those described in EP1344785.

Other methods of preparing polyalkylene substituted phenols, for example polyisobutene substituted phenols are known to the person skilled in the art, and include the methods described in EP831141.

The hydrocarbyl substituent of component (c) has an average molecular weight of 200 to 3000. Preferably it has a molecular weight of at least 225, suitably at least 250, preferably at least 275, suitably at least 300, for example at least 325 or at least 350. In some embodiments the hydrocarbyl

substituent of component (c) has an average molecular weight of at least 375, preferably at least 400, suitably at least 475, for example at least 500.

In some embodiments component (c) may include a hydrocarbyl substituent having an average molecular weight of up to 2800, preferably up to 2600, for example up to 2500 or up to 2400.

In some embodiments the hydrocarbyl substituent of component (c) has an average molecular weight of from 400 to 2500, for example from 450 to 2400, preferably from 500 to 1500, suitably from 550 to 1300.

In some embodiments the hydrocarbyl substituent of component (c) has an average molecular weight of from 200 to 600.

In some embodiments the hydrocarbyl substituent of component (c) has an average molecular weight of from 500 to 1000.

In some embodiments the hydrocarbyl substituent of component (c) has an average molecular weight of from 700 to 1300.

In some embodiments the hydrocarbyl substituent of component (c) has an average molecular weight of from 1000 to 2000.

In some embodiments the hydrocarbyl substituent of component (c) has an average molecular weight of from 1700 to 2600, for example 2000 to 2500.

Unless otherwise mentioned all average molecular weights referred to herein are number average molecular weights.

Components (a), (b) and (c) used to prepare the Mannich product additives of the present invention may each comprise a mixture of compounds and/or a mixture of isomers.

To form the Mannich additive of the present invention components (a) and (b) are preferably reacted in a molar ratio of 2.2-1.1:1 (aldehyde:amine), preferably 2.2-1.2:1 more preferably 2.2-1.4:1, suitably 2.1-1.5:1, preferably 2.05-1.55:1, preferably 2.1-1.6:1, suitably 1.95-1.65:1, for example 1.9-1.7:1.

The molar ratio of component (a) to component (b) (aldehyde:amine) in the reaction mixture is preferably at least 1.4:1. Suitably it is at least 1.5:1 at least 1.6:1, preferably at least 1.65:1, for example at least 1.7:1 or at least 1.75:1.

The molar ratio of component (a) to component (b) (aldehyde:amine) in the reaction mixture is preferably up to 2.2:1. Preferably it is up to 2.1:1, more preferably up to 2:1, suitably up to 1.95:1, for example up to 1.9:1 or up to 1.85:1.

To form a preferred Mannich additive of the present invention the molar ratio of component (a) to component (c) (aldehyde:phenol) in the reaction mixture is preferably 1.95-1.05:1, preferably 1.9-1.05:1, more preferably 1.8-1.1:1, suitably 1.7-1.1:1, preferably 165-1.15:1, more preferably 1.6-1.2:1, suitably 1.55-1.25:1, for example 1.5-1.3:1.

The molar ratio of component (a) to component (c) (aldehyde:phenol) in the reaction mixture used to prepare the Mannich additive of the present invention is preferably at least 1:1. Preferably it is at least 1.1:1, suitably at least 1.15:1, preferably at least 1.2:1, more preferably at least 1.25:1, for example at least 1.3:1.

The molar ratio of component (a) to component (c) (aldehyde:phenol) is preferably up to 1.8:1. Preferably it is up to 1.7:1; preferably up to 1.65:1, suitably up to 1.6:1, preferably up to 1.55:1, for example up to 1.5:1.

Suitably the molar ratio of component (b) to component (c) (amine:phenol) in the reaction mixture used to prepare the Mannich additive is 1:1.05-1.95, preferably 1:1.05-1.9, more preferably 1:1.05-1.8, suitably 1:1.1-1.7, preferably from 1:1.1-1.6, suitably 1:1.15-1.5, preferably 1:1.15-1.45, for example 1:1.2-1.4.

The molar ratio of component (c) to component (b) (phenol:amine) is preferably up to 2:1. It may be up to 1.9:1, suitably up to 1.8:1, preferably up to 1.7:1, more preferably up to 1.6:1, preferably up to 1.5:1, for example up to 1.45:1 or up to 1.4:1.

The molar ratio of component (c) to component (b) (phenol to amine) is preferably at least 1:1. It may be at least 1.05:1, preferably at least 1.1:1, more preferably at least 1.15:1, for example at least 1.2:1.

In some preferred embodiments in the reaction used to make the Mannich additive of the present invention the molar ratio of component (a) to component (b) is 2-1.6:1, the molar ratio of component (a) to component (c) is 1.6-1.2:1 and the molar ratio of component (b) to component (c) is 1:1.1-1.5.

In some preferred embodiments in the reaction used to make the Mannich additive of the present invention the molar ratio of component (a) to component (b) is 1.9-1.7:1, the molar ratio of component (a) to component (c) is 1.5-1.3:1 and the molar ratio of component (b) to component (c) is 1:1.2-1.4.

The ratios of the components (a), (b) and (c) used in the Mannich reaction used to prepare the additives of the present invention is very important. The inventors have found that if the ratio used fall outside this range the additive is not as effective.

In some preferred embodiments the diesel fuel composition of the present invention may further comprise a quaternary ammonium salt additive. Suitably the quaternary ammonium salt additive is formed by the reaction a quaternising agent and a compound formed by the reaction of a hydrocarbyl-substituted acylating agent and an amine of formula (B1) or (B2):



wherein  $\text{R}^2$  and  $\text{R}^3$  are the same or different alkyl, alkenyl or aryl groups having from 1 to 22 carbon atoms;  $\text{X}$  is a bond or alkylenic group having from 1 to 20 carbon atoms;  $n$  is from 0 to 20;  $m$  is from 1 to 5; and  $\text{R}^4$  is hydrogen or a  $\text{C}_1$  to  $\text{C}_{22}$  alkyl group.

The quaternising agent may suitably be selected from esters and non-esters.

In some preferred embodiments quaternising agents used to form the quaternary ammonium salt additives of the present invention are esters. Preferred ester quaternising agents are compounds of formula  $\text{RCOOR}^1$  in which  $\text{R}$  is an optionally substituted alkyl, alkenyl, aryl or alkylaryl group and  $\text{R}^1$  is a  $\text{C}_1$  to  $\text{C}_{22}$  alkyl, aryl or alkylaryl group.

Suitable ester quaternising agents include esters of carboxylic acids having a  $\text{pK}_a$  of 3.5 or less.

The compound of formula  $\text{RCOOR}^1$  is preferably an ester of a carboxylic acid selected from a substituted aromatic carboxylic acid, an  $\alpha$ -hydroxycarboxylic acid and a polycarboxylic acid.

In some preferred embodiments the compound of formula  $\text{RCOOR}^1$  is an ester of a substituted aromatic carboxylic acid and thus  $\text{R}$  is a substituted aryl group.

Preferably R is a substituted aryl group having 6 to 10 carbon atoms, preferably a phenyl or naphthyl group, most preferably a phenyl group. R is suitably substituted with one or more groups selected from carboalkoxy, nitro, cyano, hydroxy, SR<sup>5</sup> or NR<sup>5</sup>R<sup>6</sup>. Each of R<sup>5</sup> and R<sup>6</sup> may be hydrogen or optionally substituted alkyl, alkenyl, aryl or carboalkoxy groups. Preferably each of R<sup>5</sup> and R<sup>6</sup> is hydrogen or an optionally substituted C<sub>1</sub> to C<sub>22</sub> alkyl group, preferably hydrogen or a C<sub>1</sub> to C<sub>16</sub> alkyl group, preferably hydrogen or a C<sub>1</sub> to C<sub>10</sub> alkyl group, more preferably hydrogen C<sub>1</sub> to C<sub>4</sub> alkyl group. Preferably R<sup>5</sup> is hydrogen and R<sup>6</sup> is hydrogen or a C<sub>1</sub> to C<sub>4</sub> alkyl group. Most preferably R<sup>5</sup> and R<sup>6</sup> are both hydrogen. Preferably R is an aryl group substituted with one or more groups selected from hydroxyl, carboalkoxy, nitro, cyano and NH<sub>2</sub>. R may be a poly-substituted aryl group, for example trihydroxyphenyl. Preferably R is a mono-substituted aryl group. Preferably R is an ortho substituted aryl group. Suitably R is substituted with a group selected from OH, NH<sub>2</sub>, NO<sub>2</sub> or COOME. Preferably R is substituted with an OH or NH<sub>2</sub> group. Suitably R is a hydroxy substituted aryl group. Most preferably R is a 2-hydroxyphenyl group.

Preferably R<sup>1</sup> is an alkyl or alkylaryl group. R<sup>1</sup> may be a C<sub>1</sub> to C<sub>16</sub> alkyl group, preferably a C<sub>1</sub> to C<sub>10</sub> alkyl group, suitably a C<sub>1</sub> to C<sub>8</sub> alkyl group. R<sup>1</sup> may be C<sub>1</sub> to C<sub>16</sub> alkylaryl group, preferably a C<sub>1</sub> to C<sub>10</sub> alkyl group, suitably a C<sub>1</sub> to C<sub>8</sub> alkylaryl group. R<sup>1</sup> may be methyl, ethyl, propyl, butyl, pentyl, benzyl or an isomer thereof. Preferably R<sup>1</sup> is benzyl or methyl. Most preferably R<sup>1</sup> is methyl.

An especially preferred compound of formula RCOOR<sup>1</sup> is methyl salicylate.

In some embodiments the compound of formula RCOOR<sup>1</sup> is an ester of an  $\alpha$ -hydroxycarboxylic acid. In such embodiments the compound has the structure:



wherein R<sup>7</sup> and R<sup>8</sup> are the same or different and each is selected from hydrogen, alkyl, alkenyl, aralkyl or aryl. Compounds of this type suitable for use herein are described in EP 1254889.

Examples of compounds of formula RCOOR<sup>1</sup> in which RCOO is the residue of an  $\alpha$ -hydroxycarboxylic acid include methyl-, ethyl-, propyl-, butyl-, pentyl-, hexyl-, benzyl-, phenyl-, and allyl esters of 2-hydroxyisobutyric acid; methyl-, ethyl-, propyl-, butyl-, pentyl-, hexyl-, benzyl-, phenyl-, and allyl esters of 2-hydroxy-2-methylbutyric acid; methyl-, ethyl-, propyl-, butyl-, pentyl-, hexyl-, benzyl-, phenyl-, and allyl esters of 2-hydroxy-2-ethylbutyric acid; methyl-, ethyl-, propyl-, butyl-, pentyl-, hexyl-, benzyl-, phenyl-, and allyl esters of lactic acid; and methyl-, ethyl-, propyl-, butyl-, pentyl-, hexyl-, allyl-, benzyl-, and phenyl esters of glycolic acid. Of the above, a preferred compound is methyl 2-hydroxyisobutyrate.

In some embodiments the compound of formula RCOOR<sup>1</sup> is an ester of a polycarboxylic acid. In this definition we mean to include dicarboxylic acids and carboxylic acids having more than 2 acidic moieties. In such embodiments RCOO is preferably present in the form of an ester, that is the one or more further acid groups present in the group R are in esterified form. Preferred esters are C<sub>1</sub> to C<sub>4</sub> alkyl esters.

The ester quaternising agent may be selected from the diester of oxalic acid, the diester of phthalic acid, the diester

of maleic acid, the diester of malonic acid or the diester of citric acid. One especially preferred compound of formula RCOOR<sup>1</sup> is dimethyl oxalate.

In preferred embodiments the compound of formula RCOOR<sup>1</sup> is an ester of a carboxylic acid having a pK<sub>a</sub> of less than 3.5. In such embodiments in which the compound includes more than one acid group, we mean to refer to the first dissociation constant.

The ester quaternising agent may be selected from an ester of a carboxylic acid selected from one or more of oxalic acid, phthalic acid, salicylic acid, maleic acid, malonic acid, citric acid, nitrobenzoic acid, aminobenzoic acid and 2,4,6-trihydroxybenzoic acid.

Preferred ester quaternising agents include dimethyl oxalate, methyl 2-nitrobenzoate and methyl salicylate.

Suitable non-ester quaternising agents include dialkyl sulfates, benzyl halides, hydrocarbyl substituted carbonates, hydrocarbyl substituted epoxides in combination with an acid, alkyl halides, alkyl sulfonates, sultones, hydrocarbyl substituted phosphates, hydrocarbyl substituted borates, alkyl nitrates, alkyl nitrates, hydroxides, N-oxides or mixtures thereof.

In some embodiments the quaternary ammonium salt may be prepared from, for example, an alkyl or benzyl halide (especially a chloride) and then subjected to an ion exchange reaction to provide a different anion as part of the quaternary ammonium salt. Such a method may be suitable to prepare quaternary ammonium hydroxides, alkoxides, nitrites or nitrates.

Preferred non-ester quaternising agents include dialkyl sulfates, benzyl halides, hydrocarbyl substituted carbonates, hydrocarbyl substituted epoxides in combination with an acid, alkyl halides, alkyl sulfonates, sultones, hydrocarbyl substituted phosphates, hydrocarbyl substituted borates, N-oxides or mixtures thereof.

Suitable dialkyl sulfates for use herein as quaternising agents include those including alkyl groups having 1 to 10, preferably 1 to 4 carbons atoms in the alkyl chain. A preferred compound is dimethyl sulfate.

Suitable benzyl halides include chlorides, bromides and iodides. The phenyl group may be optionally substituted, for example with one or more alkyl or alkenyl groups, especially when the chlorides are used. A preferred compound is benzyl bromide.

Suitable hydrocarbyl substituted carbonates may include two hydrocarbyl groups, which may be the same or different. Each hydrocarbyl group may contain from 1 to 50 carbon atoms, preferably from 1 to 20 carbon atoms, more preferably from 1 to 10 carbon atoms, suitably from 1 to 5 carbon atoms. Preferably the or each hydrocarbyl group is an alkyl group. Preferred compounds of this type include diethyl carbonate and dimethyl carbonate.

Suitable hydrocarbyl substituted epoxides have the formula:



wherein each of R<sup>1</sup>, R<sup>2</sup>, R<sup>3</sup> and R<sup>4</sup> is independently hydrogen or a hydrocarbyl group having 1 to 50 carbon atoms.

Examples of suitable epoxides include ethylene oxide, propylene oxide, butylene oxide, styrene oxide and stillbene oxide. The hydrocarbyl epoxides are used as quaternising

## 11

agents in combination with an acid. In embodiments in which the hydrocarbyl substituted acylating agent is a dicarboxylic acylating agent no separate acid needs to be added. However in other embodiments an acid such as acetic acid may be used.

Especially preferred epoxide quaternising agents are propylene oxide and styrene oxide.

Suitable alkyl halides for use herein include chlorides, bromides and iodides.

Suitable alkyl sulfonates include those having 1 to 20, preferably 1 to 10, more preferably 1 to 4 carbon atoms.

Suitable sultones include propane sultone and butane sultone.

Suitable hydrocarbyl substituted phosphates include dialkyl phosphates, trialkyl phosphates and O,O-dialkyl dithiophosphates. Preferred alkyl groups have 1 to 12 carbon atoms.

Suitable hydrocarbyl substituted borate groups include alkyl borates having 1 to 12 carbon atoms.

Preferred alkyl nitrates and alkyl nitrates have 1 to 12 carbon atoms.

Preferably the non-ester quaternising agent is selected from dialkyl sulfates, benzyl halides, hydrocarbyl substituted carbonates, hydrocarbyl substituted epoxides in combination with an acid, and mixtures thereof.

Especially preferred non-ester quaternising agents for use herein are hydrocarbyl substituted epoxides in combination with an acid. These may include embodiments in which a separate acid is provided or embodiments in which the acid is provided by the tertiary amine compound that is being quaternised. Preferably the acid is provided by the tertiary amine molecule that is being quaternised.

Preferred quaternising agents for use herein include dimethyl oxalate, methyl 2-nitrobenzoate, methyl salicylate and styrene oxide or propylene oxide optionally in combination with an additional acid.

To form the quaternary ammonium salt additives of the present invention the quaternising agent is reacted with a compound formed by the reaction of a hydrocarbyl substituted acylating agent and an amine of formula (B1) or (B2).

When a compound of formula (B1) is used, R<sup>4</sup> is preferably hydrogen or a C<sub>1</sub> to C<sub>16</sub> alkyl group, preferably a C<sub>1</sub> to C<sub>10</sub> alkyl group, more preferably a C<sub>1</sub> to C<sub>6</sub> alkyl group. When R<sup>4</sup> is alkyl it may be straight chained or branched. It may be substituted for example with a hydroxy or alkoxy substituent. Preferably R<sup>4</sup> is not a substituted alkyl group. Preferably R<sup>4</sup> is selected from hydrogen, methyl, ethyl, propyl, butyl and isomers thereof. Most preferably R<sup>4</sup> is hydrogen.

When a compound of formula (B2) is used, m is preferably 2 or 3, most preferably 2; n is preferably from 0 to 15, preferably 0 to 10, more preferably from 0 to 5. Most preferably n is 0 and the compound of formula (B2) is an alcohol.

Preferably the hydrocarbyl substituted acylating agent is reacted with a diamine compound of formula (B1).

R<sup>2</sup> and R<sup>3</sup> are the same or different alkyl, alkenyl or aryl groups having from 1 to 22 carbon atoms. In some embodiments R<sup>2</sup> and R<sup>3</sup> may be joined together to form a ring structure, for example a piperidine or imidazole moiety. R<sup>2</sup> and R<sup>3</sup> may be branched alkyl or alkenyl groups. Each may be substituted, for example with a hydroxy or alkoxy substituent.

Preferably R<sup>2</sup> and R<sup>3</sup> is each independently a C<sub>1</sub> to C<sub>16</sub> alkyl group, preferably a C<sub>1</sub> to C<sub>10</sub> alkyl group. R<sup>2</sup> and R<sup>3</sup> may independently be methyl, ethyl, propyl, butyl, pentyl, hexyl, heptyl, octyl, or an isomer of any of these. Preferably R<sup>2</sup> and R<sup>3</sup> is each independently C<sub>1</sub> to C<sub>4</sub> alkyl. Preferably R<sup>2</sup> is methyl. Preferably R<sup>3</sup> is methyl.

X is a bond or alkylene group having from 1 to 20 carbon atoms. In preferred embodiments when X alkylene group this

## 12

group may be straight chained or branched. The alkylene group may include a cyclic structure therein. It may be optionally substituted, for example with a hydroxy or alkoxy substituent.

5 X is preferably an alkylene group having 1 to 16 carbon atoms, preferably 1 to 12 carbon atoms, more preferably 1 to 8 carbon atoms, for example 2 to 6 carbon atoms or 2 to 5 carbon atoms. Most preferably X is an ethylene, propylene or butylene group, especially a propylene group.

10 Examples of compounds of formula (B1) suitable for use herein include 1-aminopiperidine, 1-(2-aminoethyl)piperidine, 1-(3-aminopropyl)-2-pipecline, 1-methyl-(4-methylamino)piperidine, 4-(1-pyrrolidinyl)piperidine, 1-(2-aminoethyl)pyrrolidine, 2-(2-aminoethyl)-1-methylpyrrolidine, N,N-diethylethylenediamine, N,N-dimethylethylenediamine, N,N-dibutylethylenediamine, N,N-diethyl-1,3-diaminopropane, N,N,N'-trimethylmethylethylenediamine, N,N-dimethyl-N'-ethylethylenediamine, N,N,N'-triethylethylenediamine,

20 3-dimethylaminopropylamine, 3-diethylaminopropylamine, 3-dibutylaminopropylamine, N,N,N'-trimethyl-1,3-propanediamine, N,N,2,2-tetramethyl-1,3-propanediamine, 2-amino-5-diethylaminopentane, N,N,N',N'-tetraethylmethylethylenetriamine, 3,3'-diamino-N-methyldipropylamine, 3,3'-iminobis(N,N-dimethylpropylamine), 1-(3-aminopropyl)imidazole and 4-(3-aminopropyl)morpholine, 1-(2-aminoethyl)piperidine, 3,3-diamino-N-methyldipropylamine, 3,3-aminobis(N,N-dimethylpropylamine), or combinations thereof.

25 In some preferred embodiments the compound of formula (B1) is selected from N,N-dimethyl-1,3-diaminopropane, N,N-diethyl-1,3-diaminopropane, N,N-dimethylethylenediamine, N,N-diethylethylenediamine, N,N-dibutylethylenediamine, or combinations thereof.

30 Examples of compounds of formula (B2) suitable for use herein include alkanolamines including but not limited to triethanolamine, N,N-dimethylaminopropanol, N,N-diethylaminopropanol, N,N-diethylaminobutanol, triisopropanolamine, 1-[2-hydroxyethyl]piperidine, 2-[2-(dimethylamine)ethoxy]-ethanol, N-ethylidiethanolamine, N-methylidiethanolamine, N-butyldiethanolamine, N,N-diethylaminoethanol, N,N-dimethylaminoethanol, 2-dimethylamino-2-methyl-1-propanol.

35 40 In some preferred embodiments the compound of formula (B2) is selected from Triisopropanolamine, 1-[2-hydroxyethyl]piperidine, 2-[2-(dimethylamine)ethoxy]-ethanol, N-ethylidiethanolamine, N-methylidiethanolamine, N-butyldiethanolamine, N,N-diethylaminoethanol, N,N-dimethylaminoethanol, 2-dimethylamino-2-methyl-1-propanol, or combinations thereof.

45 50 An especially preferred compound of formula (B1) is dimethylaminopropylamine.

55 The amine of formula (B1) or (B2) is reacted with a hydrocarbyl substituted acylating agent. The hydrocarbyl substituted acylating agent may be based on a hydrocarbyl substituted mono-di- or polycarboxylic acid or a reactive equivalent thereof. Preferably the hydrocarbyl substituted acylating agent is a hydrocarbyl substituted succinic acid compound such as a succinic acid or succinic anhydride.

60 The hydrocarbyl substituent preferably comprises at least 10, more preferably at least 12, for example 30 or 50 carbon atoms. It may comprise up to about 200 carbon atoms. Preferably the hydrocarbyl substituent has a number average molecular weight (M<sub>n</sub>) of between 170 to 2800, for example

## 13

from 250 to 1500, preferably from 500 to 1500 and more preferably 500 to 1100. An Mn of 700 to 1300 is especially preferred.

The hydrocarbyl based substituents may be made from homo- or interpolymers (e.g. copolymers, terpolymers) of mono- and di-olefins having 2 to 10 carbon atoms, for example ethylene, propylene, butane-1, isobutene, butadiene, isoprene, 1-hexene, 1-octene, etc. Preferably these olefins are 1-monoolefins. The hydrocarbyl substituent may also be derived from the halogenated (e.g. chlorinated or brominated) analogs of such homo- or interpolymers. Alternatively the substituent may be made from other sources, for example monomeric high molecular weight alkenes (e.g. 1-tetra-concane) and chlorinated analogs and hydrochlorinated analogs thereof, aliphatic petroleum fractions, for example paraffin waxes and cracked and chlorinated analogs and hydrochlorinated analogs thereof, white oils, synthetic alkenes for example produced by the Ziegler-Natta process (e.g. poly(ethylene) greases) and other sources known to those skilled in the art. Any unsaturation in the substituent may if desired be reduced or eliminated by hydrogenation according to procedures known in the art.

The term "hydrocarbyl" as used herein denotes a group having a carbon atom directly attached to the remainder of the molecule and having a predominantly aliphatic hydrocarbon character. Suitable hydrocarbyl based groups may contain non-hydrocarbon moieties. For example they may contain up to one non-hydrocarbyl group for every ten carbon atoms provided this non-hydrocarbyl group does not significantly alter the predominantly hydrocarbon character of the group. Those skilled in the art will be aware of such groups, which include for example hydroxyl, oxygen, halo (especially chloro and fluoro), alkoxy, alkyl mercapto, alkyl sulphoxy, etc. Preferred hydrocarbyl based substituents are purely aliphatic hydrocarbon in character and do not contain such groups.

The hydrocarbyl-based substituents are preferably predominantly saturated, that is, they contain no more than one carbon-to-carbon unsaturated bond for every ten carbon-to-carbon single bonds present. Most preferably they contain no more than one carbon-to-carbon unsaturated bond for every 50 carbon-to-carbon bonds present.

Preferred hydrocarbyl-based substituents are poly(isobutene)s known in the art. Thus in especially preferred embodiments the hydrocarbyl substituted acylating agent is a polyisobutetyl substituted succinic anhydride.

The preparation of polyisobutetyl substituted succinic anhydrides (PIBSA) is documented in the art. Suitable processes include thermally reacting polyisobutenes with maleic anhydride (see for example U.S. Pat. No. 3,361,673 and U.S. Pat. No. 3,018,250), and reacting a halogenated, in particular a chlorinated, polyisobutene (PIB) with maleic anhydride (see for example U.S. Pat. No. 3,172,892). Alternatively, the polyisobutetyl succinic anhydride can be prepared by mixing the polyolefin with maleic anhydride and passing chlorine through the mixture (see for example GB-A-949,981).

Conventional polyisobutenes and so-called "highly-reactive" polyisobutenes are suitable for use in preparing additive (i) of the present invention. Highly reactive polyisobutenes in this context are defined as polyisobutenes wherein at least 50%, preferably 70% or more, of the terminal olefinic double bonds are of the vinylidene type as described in EP0565285. Particularly preferred polyisobutenes are those having more than 80 mol % and up to 100% of terminal vinylidene groups such as those described in EP1344785.

## 14

Other preferred hydrocarbyl groups include those having an internal olefin for example as described in the applicant's published application WO2007/015080.

An internal olefin as used herein means any olefin containing predominantly a non-alpha double bond, that is a beta or higher olefin. Preferably such materials are substantially completely beta or higher olefins, for example containing less than 10% by weight alpha olefin, more preferably less than 5% by weight or less than 2% by weight. Typical internal olefins include Neodene 1518IO available from Shell.

Internal olefins are sometimes known as isomerised olefins and can be prepared from alpha olefins by a process of isomerisation known in the art, or are available from other sources. The fact that they are also known as internal olefins reflects that they do not necessarily have to be prepared by isomerisation.

Some preferred acylating agents for use in the preparation of the quaternary ammonium salt additives of the present invention are polyisobutene-substituted succinic acids or succinic anhydrides. When a compound of formula (B2) is reacted with a succinic acylating agent the resulting product is a succinic ester. When a succinic acylating agent is reacted with a compound of formula (B1) in which R<sup>4</sup> is hydrogen the resulting product may be a succinimide or a succinamide. When a succinic acylating agent is reacted with a compound of formula (B1) in which R<sup>4</sup> is not hydrogen the resulting product is an amide.

In preferred embodiments, the reaction product of the hydrocarbyl substituted acylating agent and the amine of formula (B1) or (B2) is an amide or an ester.

In preferred embodiments, the reaction product of the hydrocarbyl substituted acylating agent and the amine of formula (B1) or (B2) also has at least one remaining carboxylic acid group. This may be achieved by choosing hydrocarbyl substituted acylating agents having di or polycarboxylic acids or reactive equivalents thereof and by choosing suitable molar ratios of amines of formula (B1) or (B2). In the case of amides prepared from amines of formula (B2) where R<sup>4</sup> is hydrogen, it may also be necessary to control the reaction conditions to avoid forming imides. Such techniques are within the capability of someone of ordinary skill in the art.

For the avoidance of doubt, succinic esters include the monoester compounds having the general formula (C1) and the diester compounds having the general formula (C2); succinimides have the general formula (C3); and succinamides include the monoamide compounds having the general formula (C4) and the diamide compounds having the general formula (C5):



15

-continued



16

Suitably the quaternary ammonium salt additive is present in the diesel fuel composition in an amount of from 1 to 10000 ppm, preferably from 1 to 1000 ppm, more preferably from 5 to 500 ppm, suitably from 5 to 250 ppm, for example from 5 to 150 ppm.

The weight ratio of the quaternary ammonium salt additive to the Mannich additive is preferably from 1:10 to 10:1, preferably from 1:4 to 4:1, for example from 1:3 to 3:1.

As stated previously, fuels containing biodiesel or metals 10 are known to cause fouling. Severe fuels, for example those containing high levels of metals and/or high levels of biodiesel may require higher treat rates of the quaternary ammonium salt additive and/or Mannich additive than fuels which are less severe.

15 The diesel fuel composition of the present invention may include one or more further additives such as those which are 20 commonly found in diesel fuels. These include, for example, antioxidants, dispersants, detergents, metal deactivating compounds, wax anti-settling agents, cold flow improvers, 25 cetane improvers, dehazers, stabilisers, demulsifiers, anti-foams, corrosion inhibitors, lubricity improvers, dyes, markers, combustion improvers, metal deactivators, odour masks, drag reducers and conductivity improvers. Examples of suitable amounts of each of these types of additives will be known 30 to the person skilled in the art.

In some preferred embodiments the composition additionally comprises a detergent of the type formed by the reaction of a polyisobutene-substituted succinic acid-derived acylating agent and a polyethylene polyamine. Suitable compounds 35 are, for example, described in WO2009/040583.

By diesel fuel we include any fuel suitable for use in a diesel engine, either for road use or non-road use. This includes, but is not limited to, fuels described as diesel, marine diesel, heavy fuel oil, industrial fuel oil etc.

35 The diesel fuel composition of the present invention may comprise a petroleum-based fuel oil, especially a middle distillate fuel oil. Such distillate fuel oils generally boil within the range of from 110° C. to 500° C., e.g. 150° C. to 400° C. The diesel fuel may comprise atmospheric distillate or 40 vacuum distillate, cracked gas oil, or a blend in any proportion of straight run and refinery streams such as thermally and/or catalytically cracked and hydro-cracked distillates.

The diesel fuel composition of the present invention may 45 comprise Fischer-Tropsch fuels. It may comprise non-renewable Fischer-Tropsch fuels such as those described as GTL (gas-to-liquid) fuels, CTL (coal-to-liquid) fuels and OTL (oil sands-to-liquid).

The diesel fuel composition of the present invention may 50 comprise a renewable fuel such as a biofuel composition or biodiesel composition.

The diesel fuel composition may comprise 1st generation biodiesel. First generation biodiesel contains esters of, for example, vegetable oils, animal fats and used cooking fats. This form of biodiesel may be obtained by transesterification 55 of oils, for example rapeseed oil, soybean oil, safflower oil, palm 25 oil, corn oil, peanut oil, cotton seed oil, tallow, coconut oil, physic nut oil (*Jatropha*), sunflower seed oil, used cooking oils, hydrogenated vegetable oils or any mixture thereof, with an alcohol, usually a monoalcohol, in the presence of a catalyst.

The diesel fuel composition may comprise second generation biodiesel. Second generation biodiesel is derived from renewable resources such as vegetable oils and animal fats and processed, often in the refinery, often using hydroprocessing such as the H-Bio process developed by Petrobras. 60 Second generation biodiesel may be similar in properties and quality to petroleum based fuel oil streams, for example

In especially preferred embodiments the quaternary ammonium salt additives of the present invention are salts of tertiary amines prepared from dimethylamino propylamine and a polyisobutylene-substituted succinic anhydride. The average molecular weight of the polyisobutylene substituent is preferably from 700 to 1300, more preferably from 900 to 1100.

Particularly preferred quaternary ammonium salts of the present invention are the reaction product of a polyisobutylene succinic acylating agent with dimethylaminopropylamine (N,N dimethyl 1,3 propane diamine) to form either the imide and then quaternised using methyl salicylate, or to form the half amide, half acid and then quaternised using propylene oxide.

The quaternary ammonium salt additives of the present invention may be prepared by any suitable methods. Such methods will be known to the person skilled in the art and are exemplified herein. Typically the quaternary ammonium salt additives will be prepared by heating the quaternising agent and a compound prepared by the reaction of a hydrocarbyl substituted acylating agent with an amine of formula (B1) or (B2) in an approximate 1:1 molar ratio, optionally in the presence of a solvent. The resulting crude reaction mixture may be added directly to a diesel fuel, optionally following removal of solvent. Any by-products or residual starting materials still present in the mixture have not been found to cause any detriment to the performance of the additive. Thus the present invention may provide a diesel fuel composition comprising the reaction product of a quaternising agent and the reaction product of a hydrocarbyl substituted acylating agent and an amine formula (B1) or (B2).

Suitable treat rates of the mannich additive and when present the quaternary ammonium salt additive will depend on the desired performance and on the type of engine in which they are used. For example different levels of additive may be needed to achieve different levels of performance.

Suitably the Mannich additive when used is present in the diesel fuel composition in an amount of from 1 to 10000 ppm, preferably from 1 to 1000 ppm, more preferably from 5 to 500 ppm, suitably from 5 to 250 ppm, for example from 5 to 150 ppm.

renewable diesel produced from vegetable oils, animal fats etc. and marketed by ConocoPhillips as Renewable Diesel and by Neste as NExBTL.

The diesel fuel composition of the present invention may comprise third generation biodiesel. Third generation biodiesel utilises gasification and Fischer-Tropsch technology including those described as BTL (biomass-to-liquid) fuels. Third generation biodiesel does not differ widely from some second generation biodiesel, but aims to exploit the whole plant (biomass) and thereby widens the feedstock base.

The diesel fuel composition may contain blends of any or all of the above diesel fuel compositions.

In some embodiments the diesel fuel comprises a Fischer Tropsch fuel and/or biodiesel.

In some embodiments the diesel fuel composition of the present invention may be a blended diesel fuel comprising bio-diesel. In such blends the bio-diesel may be present in an amount of, for example up to 0.5%, up to 1%, up to 2%, up to 3%, up to 4%, up to 5%, up to 10%, up to 20%, up to 30%, up to 40%, up to 50%, up to 60%, up to 70%, up to 80%, up to 90%, up to 95% or up to 99%.

In some embodiments the diesel fuel composition may comprise a secondary fuel, for example ethanol. Preferably however the diesel fuel composition does not contain ethanol.

The diesel fuel composition of the present invention may contain a relatively high sulphur content, for example greater than 0.05% by weight, such as 0.1% or 0.2%.

However in preferred embodiments the diesel fuel has a sulphur content of at most 0.05% by weight, more preferably of at most 0.035% by weight, especially of at most 0.015%. Fuels with even lower levels of sulphur are also suitable such as, fuels with less than 50 ppm sulphur by weight, preferably less than 20 ppm, for example 10 ppm or less.

Commonly when present, metal-containing species will be present as a contaminant, for example through the corrosion of metal and metal oxide surfaces by acidic species present in the fuel or from lubricating oil. In use, fuels such as diesel fuels routinely come into contact with metal surfaces for example, in vehicle fuelling systems, fuel tanks, fuel transportation means etc. Typically, metal-containing contamination may comprise transition metals such as zinc, iron and copper; group I or group II metals such as sodium; and other metals such as lead.

In addition to metal-containing contamination which may be present in diesel fuels there are circumstances where metal-containing species may deliberately be added to the fuel. For example, as is known in the art, metal-containing fuel-borne catalyst species may be added to aid with the regeneration of particulate traps. Such catalysts are often based on metals such as iron, cerium, Group I and Group II metals e.g., calcium and strontium, either as mixtures or alone. Also used are platinum and manganese. The presence of such catalysts may also give rise to injector deposits when the fuels are used in diesel engines having high pressure fuel systems.

Metal-containing contamination, depending on its source, may be in the form of insoluble particulates or soluble compounds or complexes. Metal-containing fuel-borne catalysts are often soluble compounds or complexes or colloidal species.

In some embodiments, the metal-containing species comprises a fuel-borne catalyst.

In some embodiments, the metal-containing species comprises zinc.

In one preferred embodiment the diesel fuel composition of the invention comprises a fuel-borne catalyst which includes a metal selected from iron, cerium, group I and group

II metals, platinum, manganese and mixtures thereof. Preferred group I and group II metals include calcium and strontium.

Typically, the amount of metal-containing species in the diesel fuel, expressed in terms of the total weight of metal in the species, is between 0.1 and 50 ppm by weight, for example between 0.1 and 10 ppm by weight, based on the weight of the diesel fuel.

The fuel compositions of the present invention show improved performance when used in diesel engines having high pressure fuel systems compared with diesel fuels of the prior art.

According to a second aspect of the present invention there is provided an additive package which upon addition to a diesel fuel provides a composition of the first aspect.

The additive package may comprise a mixture of the Mannich additive, optionally the quaternary ammonium salt additive and optionally further additives, for example those described above. Alternatively the additive package may comprise a solution of additives, suitably in a mixture of hydrocarbon solvents for example aliphatic and/or aromatic solvents; and/or oxygenated solvents for example alcohols and/or ethers.

According to a third aspect of the present invention there is provided a method of operating a diesel engine, the method comprising combusting in the engine a composition of the first aspect.

According to a fourth aspect of the present invention there is provided the use of a Mannich reaction product additive as defined in relation to the first aspect in a diesel fuel composition to improve the engine performance of a diesel engine when using said diesel fuel composition.

Preferred features of the second, third and fourth aspects are as defined in relation to the first aspect.

The improvement in performance may be achieved by the reduction or the prevention of the formation of deposits in a diesel engine. This may be regarded as an improvement in "keep clean" performance. Thus the present invention may provide a method of reducing or preventing the formation of deposits in a diesel engine by combusting in said engine a composition of the first aspect.

The improvement in performance may be achieved by the removal of existing deposits in a diesel engine. This may be regarded as an improvement in "clean up" performance. Thus the present invention may provide a method of removing deposits from a diesel engine by combusting in said engine a composition of the first aspect.

In especially preferred embodiments the composition of the first aspect of the present invention may be used to provide an improvement in "keep clean" and "clean up" performance.

In some preferred embodiments the use of the third aspect may relate to the use of a quaternary ammonium salt additive, optionally in combination with a Mannich additive, in a diesel fuel composition to improve the engine performance of a diesel engine when using said diesel fuel composition wherein the diesel engine has a high pressure fuel system.

Modern diesel engines having a high pressure fuel system may be characterised in a number of ways. Such engines are typically equipped with fuel injectors having a plurality of apertures, each aperture having an inlet and an outlet.

Such modern diesel engines may be characterised by apertures which are tapered such that the inlet diameter of the spray-holes is greater than the outlet diameter.

Such modern engines may be characterised by apertures having an outlet diameter of less than 500 µm, preferably less than 200 µm, more preferably less than 150 µm, preferably less than 100 µm, most preferably less than 80 µm or less.

Such modern diesel engines may be characterised by apertures where an inner edge of the inlet is rounded.

Such modern diesel engines may be characterised by the injector having more than one aperture, suitably more than 2 apertures, preferably more than 4 apertures, for example 6 or more apertures.

Such modern diesel engines may be characterised by an operating tip temperature in excess of 250° C.

Such modern diesel engines may be characterised by a fuel pressure of more than 1350 bar, preferably more than 1500 bar, more preferably more than 2000 bar.

The use of the present invention preferably improves the performance of an engine having one or more of the above-described characteristics.

The present invention is particularly useful in the prevention or reduction or removal of deposits on injectors of engines operating at high pressures and temperatures in which fuel may be recirculated and which comprise a plurality of fine apertures through which the fuel is delivered to the engine. The present invention finds utility in engines for heavy duty vehicles and passenger vehicles. Passenger vehicles incorporating a high speed direct injection (or HSDI) engine may for example benefit from the present invention.

Within the injector body of modern diesel engines having a high pressure fuel system, clearances of only 1-2 µm may exist between moving parts and there have been reports of engine problems in the field caused by injectors sticking and particularly injectors sticking open. Control of deposits in this area can be very important.

The diesel fuel compositions of the present invention may also provide improved performance when used with traditional diesel engines. Preferably the improved performance is achieved when using the diesel fuel compositions in modern diesel engines having high pressure fuel systems and when using the compositions in traditional diesel engines. This is important because it allows a single fuel to be provided that can be used in new engines and older vehicles.

The improvement in performance of the diesel engine system may be measured by a number of ways. Suitable methods will depend on the type of engine and whether "keep clean" and/or "clean up" performance is measured.

One of the ways in which the improvement in performance can be measured is by measuring the power loss in a controlled engine test. An improvement in "keep clean" performance may be measured by observing a reduction in power loss compared to that seen in a base fuel. "Clean up" performance can be observed by an increase in power when diesel fuel compositions of the invention are used in an already fouled engine.

The improvement in performance of the diesel engine having a high pressure fuel system may be measured by an improvement in fuel economy.

The use of the third aspect may also improve the performance of the engine by reducing, preventing or removing deposits in the vehicle fuel filter.

The level of deposits in a vehicle fuel filter may be measured quantitatively or qualitatively. In some cases this may only be determined by inspection of the filter once the filter has been removed. In other cases, the level of deposits may be estimated during use.

Many vehicles are fitted with a fuel filter which may be visually inspected during use to determine the level of solids build up and the need for filter replacement. For example, one such system uses a filter canister within a transparent housing allowing the filter, the fuel level within the filter and the degree of filter blocking to be observed.

Using the fuel compositions of the present invention may result in levels of deposits in the fuel filter which are considerably reduced compared with fuel compositions not of the present invention. This allows the filter to be changed much less frequently and can ensure that fuel filters do not fail between service intervals. Thus the use of the compositions of the present invention may lead to reduced maintenance costs.

In some embodiments the occurrence of deposits in a fuel filter may be inhibited or reduced. Thus a "keep clean" performance may be observed. In some embodiments existing deposits may be removed from a fuel filter. Thus a "clean up" performance may be observed.

Improvement in performance may also be assessed by considering the extent to which the use of the fuel compositions of the invention reduce the amount of deposit on the injector of an engine. For "keep clean" performance a reduction in occurrence of deposits would be observed. For "clean up" performance removal of existing deposits would be observed.

Direct measurement of deposit build up is not usually undertaken, but is usually inferred from the power loss or fuel flow rates through the injector.

The use of the third aspect may improve the performance of the engine by reducing, preventing or removing deposits including gums and lacquers within the injector body.

In Europe the Co-ordinating European Council for the development of performance tests for transportation fuels, lubricants and other fluids (the industry body known as CEC), has developed a new test, named CEC F-98-08, to assess whether diesel fuel is suitable for use in engines meeting new European Union emissions regulations known as the "Euro 5" regulations. The test is based on a Peugeot DW10 engine using Euro 5 injectors, and will hereinafter be referred to as the DW10 test. It will be further described in the context of the examples (see example 4).

Preferably the use of the fuel composition of the present invention leads to reduced deposits in the DW10 test. For "keep clean" performance a reduction in the occurrence of deposits is preferably observed. For "clean up" performance removal of deposits is preferably observed. The DW10 test is used to measure the power loss in modern diesel engines having a high pressure fuel system.

For older engines an improvement in performance may be measured using the XUD9 test. This test is described in relation to example 9.

Suitably the use of a fuel composition of the present invention may provide a "keep clean" performance in modern diesel engines, that is the formation of deposits on the injectors of these engines may be inhibited or prevented. Preferably this performance is such that a power loss of less than 5%, preferably less than 2% is observed after 32 hours as measured by the DW10 test.

Suitably the use of a fuel composition of the present invention may provide a "clean up" performance in modern diesel engines, that is deposits on the injectors of an already fouled engine may be removed. Preferably this performance is such that the power of a fouled engine may be returned to within 1% of the level achieved when using clean injectors within 32 hours as measured in the DW10 test.

Preferably rapid "clean-up" may be achieved in which the power is returned to within 1% of the level observed using clean injectors within 10 hours, preferably within 8 hours, suitably within 6 hours, preferably within 4 hours, more preferably within 2 hours.

Clean injectors can include new injectors or injectors which have been removed and physically cleaned, for example in an ultrasound bath.

Suitably the use of a fuel composition of the present invention may provide a "keep clean" performance in traditional diesel engines, that is the formation of deposits on the injectors of these engines may be inhibited or prevented. Preferably this performance is such that a flow loss of less than 50%, preferably less than 30% is observed after 10 hours as measured by the XUD-9 test.

Suitably the use of a fuel composition of the present invention may provide a "clean up" performance in traditional diesel engines, that is deposits on the injectors of an already fouled engine may be removed. Preferably this performance is such that the flow loss of a fouled engine may be increased by 10% or more within 10 hours as measured in the XUD-9 test.

Any feature of any aspect of the invention may be combined with any other feature, where appropriate.

The invention will now be further defined with reference to the following non-limiting examples.

## EXAMPLE 1

A polyisobutene-substituted phenol was prepared as follows:

Polyisobutene having an average molecular weight of 750 (450.3 g, 0.53 mol, 1 equiv) was heated to 45-50° C. and then phenol (150.0 g, 1.59 mol, 3 equivs) was added. The turbid mixture was stirred and boron trifluoride dietherate (15.0 g, 0.10 mol, 0.18 equivs) was added in 2-3 ml aliquots over approx two hours to provide a clear orange liquid which was stirred at 45-50° C. for 5 hours. Aqueous ammonia 35% (10.5 g, 0.22 moles) was then added and the reaction mixture stirred for 30 mins. Vacuum distillation provided 81.3 g of distillate. This was stirred at 70° C. in toluene (250.3 g) for 5 mins, before adding 250.4 g of water. The layers were separated and the toluene extract was washed twice more with water. Residual water and toluene removed under vacuum to provide the product as a viscous pale yellow liquid. (510.9 g) having a toluene content of 2 wt % and a phenol content of less than 0.2 wt %.

This product was used to prepare additive A, a Mannich additive of the present invention, as follows:

PIB 750 Phenol with a residual PIB content of 5 wt % (447.8 g, 425.4 g "active" PIB phenol, 0.50 moles, 1.3 equivs) was mixed with ethylenediamine (25.3 g, 0.38 moles, 1 equiv) and Caromax 20 solvent (225.6 g). The homogenous mixture was heated to 90-95° C. 36.7% formalin (57.12 g, 0.69 moles, 1.8 equivs) was then added over 1 hr and the reaction mixture was then held at 95° C. for 1 hr. Water was removed using a Dean-Stark apparatus. Following distillation 708.3 g product was collected.

## EXAMPLE 2

## Comparative

Using methods analogous to that described in example 1, comparative Mannich reaction products not of the invention were prepared using the molar ratios of components detailed in table 1.

TABLE 1

|   | Molar equivalents of formaldehyde | Molar equivalents of ethylene diamine | Molar equivalents of PIB Phenol (PIB MW = 750) |
|---|-----------------------------------|---------------------------------------|------------------------------------------------|
| B | 2                                 | 1                                     | 2                                              |
| C | 1                                 | 1                                     | 1                                              |

TABLE 1-continued

|   | Molar equivalents of formaldehyde | Molar equivalents of ethylene diamine | Molar equivalents of PIB Phenol (PIB MW = 750) |
|---|-----------------------------------|---------------------------------------|------------------------------------------------|
| D | 1                                 | 2                                     | 1                                              |
| E | 1                                 | 1                                     | 2                                              |
| F | 2                                 | 1                                     | 1                                              |

## EXAMPLE 3

Diesel fuel compositions were prepared by adding additives to aliquots all drawn from a common batch of RF06 base fuel, and containing 1 ppm zinc (as zinc neodecanoate). In each case 75 ppm of the crude additive prepared as described in examples 1 and 2 was used.

Table 2 below shows the specification for RF06 base fuel.

TABLE 2

|    | Property                            | Units                | Limits |       | Method        |
|----|-------------------------------------|----------------------|--------|-------|---------------|
|    |                                     |                      | Min    | Max   |               |
| 25 | Cetane Number                       |                      | 52.0   | 54.0  | EN ISO 5165   |
|    | Density at 15° C.                   | kg/m <sup>3</sup>    | 833    | 837   | EN ISO 3675   |
|    | Distillation                        |                      |        |       |               |
| 30 | 50% v/v Point                       | °C.                  | 245    | —     |               |
|    | 95% v/v Point                       | °C.                  | 345    | 350   |               |
|    | FBP                                 | °C.                  | —      | 370   |               |
| 35 | Flash Point                         | °C.                  | 55     | —     | EN 22719      |
|    | Cold Filter Plugging Point          | °C.                  | —      | -5    | EN 116        |
|    | Viscosity at 40° C.                 | mm <sup>2</sup> /sec | 2.3    | 3.3   | EN ISO 3104   |
| 40 | Polycyclic Aromatic                 | % m/m                | 3.0    | 6.0   | IP 391        |
|    | Hydrocarbons                        |                      |        |       |               |
|    | Sulphur Content                     | mg/kg                | —      | 10    | ASTM D 5453   |
| 45 | Copper Corrosion                    | % m/m                | —      | 1     | EN ISO 2160   |
|    | Conradson Carbon                    | % m/m                | —      | 0.2   | EN ISO 10370  |
|    | Residue on 10% Dist. Residue        |                      |        |       |               |
|    | Ash Content                         | % m/m                | —      | 0.01  | EN ISO 6245   |
|    | Water Content                       | % m/m                | —      | 0.02  | EN ISO 12937  |
| 50 | Neutralisation (Strong Acid) Number | mg KOH/g             | —      | 0.02  | ASTM D 974    |
|    | Oxidation Stability                 | mg/mL                | —      | 0.025 | EN ISO 12205  |
|    | HFRR (WSD1, 4)                      | μm                   | —      | 400   | CEC F-06-A-96 |
|    | Fatty Acid Methyl Ester             |                      |        |       | prohibited    |

## EXAMPLE 4

The performance of diesel fuel compositions of the present invention in modern diesel engines may be tested according to the CECF-98-08 DW 10 method.

The engine of the injector fouling test is the PSA DW10BTED4. In summary, the engine characteristics are:

Design: Four cylinders in line, overhead camshaft, turbocharged with EGR

Capacity: 1998 cm<sup>3</sup>

Combustion chamber: Four valves, bowl in piston, wall guided direct injection

Power: 100 kW at 4000 rpm

60 Torque: 320 Nm at 2000 rpm

Injection system: Common rail with piezo electronically controlled 6-hole injectors.

Max. pressure: 1600 bar ( $1.6 \times 10^8$  Pa). Proprietary design by SIEMENS VDO

65 Emissions control: Conforms with Euro IV limit values when combined with exhaust gas post-treatment system (DPF)

This engine was chosen as a design representative of the modern European high-speed direct injection diesel engine capable of conforming to present and future European emissions requirements. The common rail injection system uses a highly efficient nozzle design with rounded inlet edges and conical spray holes for optimal hydraulic flow. This type of nozzle, when combined with high fuel pressure has allowed advances to be achieved in combustion efficiency, reduced noise and reduced fuel consumption, but are sensitive to influences that can disturb the fuel flow, such as deposit formation in the spray holes. The presence of these deposits causes a significant loss of engine power and increased raw emissions.

The test is run with a future injector design representative of anticipated Euro V injector technology. It is considered necessary to establish a reliable baseline of injector condition before beginning fouling tests, so a sixteen hour running-in schedule for the test injectors is specified, using non-fouling reference fuel.

Full details of the CEC F-98-08 test method can be obtained from the CEC. The coking cycle is summarised below.

1. A warm up cycle (12 minutes) according to the following regime:

| Step | Duration (minutes) | Engine Speed (rpm) | Torque (Nm) |
|------|--------------------|--------------------|-------------|
| 1    | 2                  | idle               | <5          |
| 2    | 3                  | 2000               | 50          |
| 3    | 4                  | 3500               | 75          |
| 4    | 3                  | 4000               | 100         |

2. 8 hrs of engine operation consisting of 8 repeats of the following cycle

| Step | Duration (minutes) | Engine Speed (rpm) | Load (%) | Torque (Nm) | Boost Air After IC (° C.) |
|------|--------------------|--------------------|----------|-------------|---------------------------|
| 1    | 2                  | 1750               | (20)     | 62          | 45                        |
| 2    | 7                  | 3000               | (60)     | 173         | 50                        |
| 3    | 2                  | 1750               | (20)     | 62          | 45                        |
| 4    | 7                  | 3500               | (80)     | 212         | 50                        |
| 5    | 2                  | 1750               | (20)     | 62          | 45                        |
| 6    | 10                 | 4000               | 100      | *           | 50                        |
| 7    | 2                  | 1250               | (10)     | 20          | 43                        |
| 8    | 7                  | 3000               | 100      | *           | 50                        |
| 9    | 2                  | 1250               | (10)     | 20          | 43                        |
| 10   | 10                 | 2000               | 100      | *           | 50                        |
| 11   | 2                  | 1250               | (10)     | 20          | 43                        |
| 12   | 7                  | 4000               | 100      | *           | 50                        |

\* for expected range see CEC method CEC-F-98-08

3. Cool down to idle in 60 seconds and idle for 10 seconds
4. 4 hrs soak period

The standard CEC F-98-08 test method consists of 32 hours engine operation corresponding to 4 repeats of steps 1-3 above, and 3 repeats of step 4. ie 56 hours total test time excluding warm ups and cool downs.

#### EXAMPLE 5

The diesel fuel compositions prepared according to example 3 were tested according to the DW-10 test method of example 4.

In each case, a 32 hour cycle was run using new injectors and RF-06 base fuel having added thereto 1 ppm Zn (as neodecanoate) and 75 ppm of the crude additive. The power

loss over the 32 hour test period was recorded in each case. The results are shown in FIGS. 1 to 6.

#### EXAMPLE 6

The reaction product of a hydrocarbyl substituted acylating agent and a compound of formula (B1) was prepared as follows:

5 10 15 20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 91

## 25

The test engine is fitted with cleaned injectors utilising unflatted injector needles. The airflow at various needle lift positions have been measured on a flow rig prior to test. The engine is operated for a period of 10 hours under cyclic conditions.

| Stage | Time (secs) | Speed (rpm) | Torque (Nm) |
|-------|-------------|-------------|-------------|
| 1     | 30          | 1200 ± 30   | 10 ± 2      |
| 2     | 60          | 3000 ± 30   | 50 ± 2      |
| 3     | 60          | 1300 ± 30   | 35 ± 2      |
| 4     | 120         | 1850 ± 30   | 50 ± 2      |

The propensity of the fuel to promote deposit formation on the fuel injectors is determined by measuring the injector nozzle airflow again at the end of test, and comparing these values to those before test. The results are expressed in terms of percentage airflow reduction at various needle lift positions for all nozzles. The average value of the airflow reduction at 0.1 mm needle lift of all four nozzles is deemed the level of injector coking for a given fuel.

The invention claimed is:

1. A diesel fuel composition comprising, as an additive, the product of a Mannich reaction between:

- (a) an aldehyde;
- (b) an amine; and
- (c) a substituted phenol;

wherein the phenol is substituted with at least one branched hydrocarbyl group having a molecular weight of between 200 and 3000; and wherein in the Mannich reaction used to form the additive the molar ratio of component (a) to component (b) is 1.95-1.6:1; the molar ratio of component (a) to component (c) is 1.7-1.1:1 and the molar ratio of component (b) to component (c) is 1:1.1-1.7.

2. The diesel fuel composition according to claim 1 wherein phenol component (c) used to prepare the Mannich additive includes a poly(isobutene) derived substituent.

3. The diesel fuel composition according to claim 1 wherein in the reaction used to make the Mannich additive the molar ratio of component (b) to component (c) is 1:1.1-1.5.

4. The diesel fuel composition according to claim 1 wherein in the reaction used to make the Mannich additive the molar ratio of component (b) to component (c) is 1:1.15-1.5.

## 26

5. The diesel fuel composition according to claim 1 wherein in the reaction used to make the Mannich additive the molar ratio of component (a) to component (c) is 1.5-1.3:1.

6. The diesel fuel composition according to claim 1 wherein in the reaction used to make the Mannich additive the molar ratio of component (b) to component (c) is 1:1.2-1.4.

7. The diesel fuel composition according to claim 1 which further comprises a quaternary ammonium salt additive formed by the reaction a quaternising agent and a compound formed by the reaction of a hydrocarbyl-substituted acylating agent and an amine of formula (B1) or (B2):

(B1)



(B2)



wherein R<sup>2</sup> and R<sup>3</sup> are the same or different alkyl, alkenyl or aryl groups having from 1 to 22 carbon atoms; X is a bond or alkylene group having from 1 to 20 carbon atoms; n is from 0 to 20; m is from 1 to 5; and R<sup>4</sup> is hydrogen or a C<sub>1</sub> to C<sub>22</sub> alkyl group.

8. The diesel fuel composition according to claim 7 wherein the quaternising agent is selected from esters, dialkyl sulfates, benzyl halides, hydrocarbyl substituted carbonates, hydrocarbyl substituted epoxides in combination with an acid, alkyl halides, alkyl sulfonates, sultones, hydrocarbyl substituted phosphates, hydrocarbyl substituted borates, alkyl nitrites, alkyl nitrates, N-oxides or mixtures thereof.

9. The diesel fuel composition according to claim 1 which further comprises a fuel-borne catalyst which includes a metal selected from iron, cerium, group I and group II metals, platinum, manganese and mixtures thereof.

10. An additive package which upon addition to a diesel fuel provides a composition as claimed in claim 1.

11. A method of operating a diesel engine, the method comprising combusting in the engine a composition as claimed in claim 1.

\* \* \* \* \*